

May 24, 1938.

E. A. HARTY

2,118,645

ELECTRIC CUT-OUT

Filed Nov. 17, 1937

Fig. 1.



Fig. 2.



Fig. 3.



Inventor:  
Edgar A. Harty,  
by Harry E. Junham  
His Attorney.

## UNITED STATES PATENT OFFICE

2,118,645

## ELECTRIC CUT-OUT

Edgar A. Harty, Marblehead, Mass., assignor to  
General Electric Company, a corporation of  
New York

Application November 17, 1937, Serial No. 174,920

5 Claims. (Cl. 200—118)

My invention relates to electric cut-outs for series circuits, and more particularly to oxide film cut-outs, the present application being a continuation in part of my application S. N. 126,031, filed 5 February 16, 1937.

One object of my invention is to provide an oxide film cut-out in which the leakage current is substantially eliminated.

For a better understanding of my invention, 10 together with other and further objects thereof, reference is had to the following description, taken in connection with the accompanying drawing, and its scope will be pointed out in the appended claims.

15 In the production of metal oxide cut-outs, it is the preferred practice to place small discs of metal, such as copper, for example, into an oxidizing atmosphere, and thereby form a coating of cuprous and cupric oxides on the surface of the 20 metal. One such process is disclosed in my U. S. Patent No. 1,982,384, issued November 27, 1934. By this process a permanent film of oxide is 25 formed on the copper disc, and when this disc is placed between two contacts, it provides a resistance to current flow up to predetermined potentials. When such predetermined potentials are exceeded, the resistance of this film breaks down and current is permitted to flow.

Some difficulty has been experienced with these 30 cut-outs due to breakdowns occurring below the rated voltage within a short time after the cut-out is placed in service. These breakdowns occur at voltages below the rated voltage, although tests indicated sufficient strength of insulation when 35 the cut-out was first put into service. Investigations have shown that considerable leakage current flows through the cut-outs when they are used on alternating current circuits. This current causes a rise in temperature in the cut-out and, 40 consequently, a deterioration of the cut-out. The probable cause of this leakage current is the unidirectional characteristic of copper oxide which is present in oxide films, treated as set forth in the above described patent, for the purpose 45 of limiting their breakdown strength to a predetermined value. Theoretically, this unidirectional characteristic should have no effect upon the cut-out as described for the reason that each disc is provided with an oxide coating on 50 both sides, thereby placing two oxide coatings in series with the current circuit in such manner that irrespective of the direction of the current flow a high resistance will be interposed in the circuit. Actually, however, slight inequalities of 55 the two opposing oxide coatings permit a small

leakage current to flow which, in the course of time, deteriorates the oxide coating and causes a breakdown thereof below the desired voltage.

I have discovered that when in the production of cut-outs, copper is used which bears a small 5 percentage of another metal, such as silver for example, the resistance to current flow in both directions, that is, in the direction of low resistance as well as in the direction of high resistance of the respective oxide coatings is materially increased 10 and a very poor rectifying ratio is obtained. I have found that this effect becomes noticeable with copper containing mere traces of silver. Satisfactory results are obtained, for example, with copper bearing silver in quantities of the order of 15 8 ounces per ton of copper. The silver, of course, need not necessarily be contained in the copper in its original state, but may be alloyed therewith at any stage of the manufacturing process, before the discs are oxidized for the purpose of converting them into cut-outs.

In the accompanying drawing, Fig. 1, I have 20 illustrated a cut-out assembled in its protective jacket and in operating position between the prongs, or terminals, of a series circuit socket; 25 in Fig. 2, I have illustrated a cross-section of the cut-out of Fig. 1; and in Fig. 3, I have indicated the relative resistance to current flow of cut-outs made with pure copper, and with copper bearing a small quantity of silver.

30 Referring to this drawing in detail, Fig. 1 illustrates the prongs 5 and 6 of a series circuit socket between which the assembled cut-out 7 provides a bar to current flow until a certain voltage is exceeded. In Fig. 2, the cut-out 7 is shown in cross-section and is shown to comprise a metal capsule 8, a cover 9 insulated therefrom by a suitable insulation 10 placed between the edge of the cover 9 and the wall of the capsule 8, the edge of the capsule being turned over to grip the cover. Contacting the inner surface of the capsule and cover is a copper disc 11, the surfaces of which are covered with an oxide film.

35 In Fig. 3, I have illustrated a graph showing the comparison between current flow through 40 pure copper discs, covered with a single film of oxide, and through oxidized discs made of silver bearing copper. Line 12 in this graph indicates the current flow, in the direction of low resistance, 45 in discs of pure copper at three volts direct current; the oxide coating being heat-treated and quenched at the temperatures indicated. The range of quenching temperatures indicated includes those that are necessary to obtain the most 50 55

commonly used breakdown voltages on cut-out discs having two opposed oxide films on opposite sides of the disc. Line 13 indicates the current flow in the low resistance direction of the oxide when copper, having mere traces of silver therein, the actual quantity being unmeasurable, and line 14 indicates current flow when copper having a silver content of the order of 8 ounces per ton is used. The relation between these three curves indicates that the oxide film loses some of its rectifying characteristics when a mere trace of silver appears in the copper and loses substantially all of this characteristic when a measurable quantity such as 8 ounces per ton, for example, is used. When two such films are opposed to each other, there is substantially no leakage current through the disc. The resistance of the disc subsequently to the breaking-down of the oxide is not materially affected by the presence of the silver in the disc.

What I claim as new and desire to secure by Letters Patent of the United States is:

1. A cut-out for electric circuits comprising an oxidized disc of copper having alloyed therewith a second metal which substantially eliminates the rectifying ratio of the oxide on said disc.
2. A cut-out for electric circuits comprising an oxidized disc of silver bearing copper.
3. A cut-out for electric circuits comprising an oxidized disc of copper, said copper bearing silver in sufficient quantity to substantially eliminate the rectifying characteristic of said disc.
4. A cut-out for electric circuits comprising an oxidized disc of copper, said copper bearing a quantity of silver of the order of 8 ounces per ton.
5. A cut-out for electric circuits comprising an oxidized copper disc, said copper having alloyed therewith silver of a quantity ranging from a mere trace up to 8 ounces per ton.

EDGAR A. HARTY. 20